

G. DEMAILLY. 2 Sheets--Sheet 1.  
Improvement in the Manufacture of Paper Pulp.  
No. 124,196. Patented March 5, 1872.



2 Sheets--Sheet 2.

G. DEMAILLY.

Improvement in the Manufacture of Paper Pulp.

No. 124,196.

Patented March 5, 1872.

FIG. 2.



12 6 9 1 8 5 4 5 Feet.

Witnesses

*A. B. B. B. B.*

Inventor.

*G. Demailly*

## UNITED STATES PATENT OFFICE.

GUSTAVE DEMAILLY, OF ARGENTEUIL, FRANCE.

## IMPROVEMENT IN THE MANUFACTURE OF PAPER-PULP.

Specification forming part of Letters Patent No. 124,196, dated March 5, 1872.

## SPECIFICATION.

I, GUSTAVE DEMAILLY, of Argenteuil, in the Empire of France, have invented certain improvements in the mode of extracting the filaments of straw and the bark of the mulberry-tree, and converting the same into pulp for the manufacture of paper, of which the following is a specification:

*Nature and Objects of the Invention.*

The first part of my invention relates to a chemical operation for preparing the filaments before submitting them to a mechanical process for converting them into pulp.

The chemical operation is as follows: Having previously cut the straw into lengths of from five to six centimeters, it is boiled in caustic lye, of from one to two degrees, for about two hours; it is then withdrawn and washed in either hot or cold water mixed with about one per cent. of sulphuric acid, in order to remove the coloring matter produced by the effect of the caustic lye. In preparing the bark of the mulberry-tree, a simple water retting will suffice when the tree is not green; or, if it is desired to accelerate the work, it may be cut in lengths of from eight to ten centimeters and boiled for a quarter of an hour in a soda-lye at one-half a degree, when it may be withdrawn and passed to the machine for converting it into pulp.

*Description of the Drawing.*

Figure 1 is a vertical section of the apparatus employed. Fig. 2 is a sectional end view of the same.

A is a grooved cylinder, turning round its axis  $o$ , and moves in a trough, B, formed of plates, also grooved, and whose circumference does not exceed that of the cylinder by more than three centimeters, and leaving between them a space determined by the nature of the substance to be treated, and the state to which it is to be reduced. These plates are maintained against the cylinder A by means of India rubbers C, fixed by one of their extremities to a transverse shaft, a, furnished at its ends with pivots, receiving rollers, rolling on an inclined plane, p. These India rubbers embrace the whole of the plates, and wind on

a second transverse shaft, a', also rolling on an inclined plane, p', and are fixed by means of iron hooks E to the levers F, supplied with weights P for regulating the pressure. The two inclined planes p p' tend to draw the extreme plates against the bars on which the India rubbers rest. On each side of the cylinder A are placed, as close as possible, two cast-iron cheeks, J J, on which are fixed parts of circular crowns of sheet-iron, D, pierced with as many rectangular guides as there are plates. These guides impart to the plates B a percussive motion, and prevent them rising one on the other. A space, which may vary from one to five-tenths of a millimeter, is made between the plates B and the cylinder A, according as it is desired to make paper-pulp, or simply to extract the filaments.

Having thus described the parts of the machine, I will now explain the *modus operandi*. The matter, having undergone the chemical process before mentioned, is spread on the endless cloth T, which leads it between the grooved cylinders M M, which latter distribute it uniformly to the machine, and force it to pass through the entrance r; it is then drawn along by the grooved cylinder A, and reaches the first plate, which, yielding to the pressure, strikes the matter, which, continuing to arrive, is treated similarly by each blade in succession. From this it will be observed that the drawing movement of the cylinder A, in conjunction with the striking of the plates, causes the separation of the filaments and the gummy particles, destroys the parenchyma, which escapes through the interstices of the grooved plates B, and effects a partial solution of the gum in the water contained in the basin b. The matter leaves the machine by the opening N in the form of filamentous rolls, and, falling on the endless cloth T, is thence conducted to an agitator, where it is separated, and is then in a condition to be employed either in the formation of tissue, (in the case of the mulberry-bark,) or for conversion into paper-pulp. In reducing the straw at once into pulp, the cylinder is completely surrounded with grooved plates; in this case the straw falls through the interstices of the plates into the lower basin b, whence it has a continuous or intermittent flow. As regards the bark, after having sub-

mitted to one machine for extracting the filaments, it is subjected to a second, completely surrounded with grooved plates, which reduce it to paste. The extraction of these latter filaments requires grooves of from four to six millimeters, and one part flat of five-tenths of a millimeter at the angle. For the manufacture of pulp, the grooves are from two to four millimeters, with the angles as sharp as possible.

*Claim.*  
I claim as my invention—

The rotary grooved cylinder with grooved blades, the India rubbers for the distribution of pressure, the iron cheeks and guides to the grooved plates, and the chemical process for preparing the filaments before submitting them to the machine, substantially as and for the purposes herein set forth.

GUSTAVE DEMAILLY.

Witnesses:

C. BLÉTRES,  
A. BLÉTRES.